

A. F. HOFFMAN.  
PROCESS FOR RECOVERING SULFUR.  
APPLICATION FILED APR. 8, 1916.

1,273,370.

Patented July 23, 1918.



**WITNESSES**

C. R. Hardy  
B. Bricard

14

Richard Oliver.

ATTORNEY

# UNITED STATES PATENT OFFICE.

ADDISON F. HOFFMAN, OF PITTSBURGH, PENNSYLVANIA.

## PROCESS FOR RECOVERING SULFUR.

1,273,370.

Specification of Letters Patent. Patented July 23, 1918.

Application filed April 8, 1916. Serial No. 39,967.

To all whom it may concern:

Be it known that I, ADDISON F. HOFFMAN, a citizen of the United States, residing at Pittsburgh, in the county of Allegheny and 5 State of Pennsylvania, have invented certain new and useful Improvements in Processes for Recovering Sulfur, of which the following is a specification.

My invention relates to a process for 10 recovering sulfur and ore from metallic sulfids or pyrites such as are usually wasted in connection with mining of coal.

It is a known fact that most of these sulfids contain approximately one-half sulfur 15 and therefore the primary object of the present process consists in the recovery of the sulfur from the above mentioned sulfids, the ore being a by product of the process.

With the above and other objects in view, 20 I will now proceed to describe my process in connection with the preferred form of apparatus for carrying out the same.

Figure 1, is a diagrammatic view illustrating the elements of the apparatus in 25 which my process is carried out, and Fig. 2, is a view in section of a retort chamber.

The apparatus as shown in the accompanying drawing consists of the retort A having the chamber B closed at the top by 30 the cover C and the opening at the bottom provided with grates D. This opening leads into a pit E in which a screw conveyer F works, such conveyer being driven by any suitable means such as G. This conveyer 35 dumps onto a second conveyer H which may be of any suitable bucket type to relieve the conveyer F of its material and remove the same from the vicinity of the retort. The back of the retort is apertured as at I and 40 covered by a door J provided with suitable air holes which may be plugged if desired. Through this aperture I the combustion in the retort may be started. Further apertures K are provided which communicate 45 with a passage L closed by an observation door M. Both the passage L and steam pipe N enter the chamber B. At the top of the retort chamber B the conduit O leads out and terminates in the conoidal top P of the 50 collector Q provided with the opening R through which contents thereof may be removed. The top P of the collector Q is provided with an outlet conduit S which leads into the bottom of a condenser and washer 55 T, said washer being closed at the bottom by door U and at the top by door V. This

washer is filled with coke or stone W which may be sprinkled with water through the medium of the sprinkler head X supplied by pipe Y. At the bottom the condenser 60 and washer T is provided with a grating Z directly over a pit A' which is relieved of its contents through a suitable conveyer B' having buckets C'. The operation of the apparatus is as follows: 65

Suppose the retort chamber B is to be charged with a metallic sulfid having the chemical formula  $FeS_2$  and that combustion is started in the presence of ample oxygen. The reaction taking place will be as fol- 70 lows:



Thus oxid of iron remains after reaction and the vapors given off are sulfur dioxid. 75 The sulfur dioxid is conveyed through the conduit O to the dust collector Q which separates any dust from the gases, and thence the vapors proceed to the condenser and washer T where they are acted on by the 80 water and a little of the sulfur dioxid dissolved in the water produces sulfurous acid. The continuance of the process is regulated by the speed of the conveyer F which regulates the rate of combustion within the re- 85 tort B. That is to say, as the refuse or metallic oxid is removed at the bottom the combustion progresses within the retort chamber B and thus the rapidity with which the process proceeds is regulated and con- 90 trolled completely by means of controlling the speed of the screw conveyer F. Of course, however, it will be necessary to employ a pyrometer to regulate the heat of combustion and means to regulate the introduction of air since the temperature of the retort chamber should, in no instance, be allowed to reach or exceed  $900^{\circ} C.$  for should it reach such a temperature the sulfids would 95 fuse. 100

When the sulfids are charged into retort chamber B, provided sufficient oxygen is not present to assist combustion to the extent indicated in the previous paragraphs, the following reaction may take place: 105



It will be seen by this reaction that the metallic oxid remains while sulfur dioxid and pure sulfur fumes pass over. 110

In treating pure pyrites such as contains 53.3% sulfur and 46.7% iron the combus-

tion will take place without the addition of fuel once the fire is started as this compound has approximately three-eighths the fuel value of coal. However, with pyrite 5 of the kind occurring along with coal in masses and bands it is impracticable to first clean it and then burn it as it usually contains a little coal and therefore the same is used in its original form since the coal 10 burns and leaves comparatively little ash in no way interfering with the process. Of course a little sulfur may unite with carbon monoxid under certain conditions to form carbon COS, but this is more than 15 compensated for by a subsequent reaction which occurs and which follows:



20 The carbonate of iron formed decomposes lower down in the retort and the effect of the small amount of coal clinging to marcasite pyrite is to produce an increase in the quantity of sulfur discharged, the quantity 25 of sulfur discharged being in the neighborhood of 60% in the form of sulfur gas and 40% sulfur dioxid. With marcasite pyrite the quantity of coal adhering to the pyrite is usually in the neighborhood of 10 and 30 15% and since sulfur volatilizes at 450° C. and distils from a metallic sulfid at approximately 700° C. the temperature of the retort chamber B must be held within the range indicated, and as before stated must 35 in no instance reach or exceed 900° C. To hold the retort chamber B within the proper temperature limits the oxygen supply must be carefully regulated and a pyrometer is absolutely essential.

40 In carrying out this process steam may be admitted to the retort B as indicated in the drawings of the apparatus and the addition of this steam acts differently according to the temperature of the retort at the 45 time of admission. If the retort chamber B is operated at a temperature above 700° C. the pyrite can be almost completely desulfurized by the use of steam, usually only 1 to 3% of sulfur remaining in the ores, whereas 50 the gas given off will consist principally of sulfur vapors, carbon dioxid, nitrogen, carbon monoxid, sulfur dioxid and hydrogen sulfid. In carrying out the process with the use of steam the following reactions may occur when the temperature of the retort chamber B is below 700° C.



60 If the gases escaping from the retort are conducted to the collector Q and thence into the condensing tower T the sulfur will be condensed and any sulfur dioxid present will combine with the hydrogen sulfid in the 65 presence of a water spray. If desired to ac-

celerate the combination in the presence of the water spray the latter may contain a catalyzing salt such as calcium chlorid the reaction taking place in the presence of the catalyzing agent will be as follows:



However, when the temperature of the retort B is above 700° C. another reaction than that above mentioned will occur since 75 in this case the iron in the sulfid will almost instantly decompose water vapor admitted or present naturally and the reaction taking place will be as follows:



80

This is due to the fact that the affinity of iron at this temperature is greater for oxygen than for sulfur or that of hydrogen for sulfur, thus the hydrogen set free will unite 85 with oxygen in preference to sulfur. The union of hydrogen and oxygen occurring higher up in the retort increases the area of high temperature to a considerable extent and the retort may be so controlled that 90 practically no sulfur is discharged as sulfureted hydrogen or sulfur dioxid, or the gases discharged may consist of sulfur, sulfur dioxid, or hydrogen sulfid which are capable of being united outside of the retort 95 in any one of several well known ways. The object of combining the various steps hereinbefore enumerated is to increase the quantity of sulfur obtained. Attention is called to the fact that no fuel is used except that which is present as a natural constituent of the raw material to be treated.

In connection with the operation of the apparatus, other than the retort, it is pointed out that the collector Q is preferably a 105 metallic barrel lined with brick so as to minimize corrosion and maintain the temperature of the gases so that the sulfur may not be condensed at this particular point in the process. The condenser or washer is so arranged that the gases enter at the bottom and progress upwardly through the material contained therein and are met by the spray. This part of the apparatus is preferably a metal cylindrical stack.

110

If instead of adding steam to the retort it is desired to carry out the process in another way the pyrite or marcasite may be burned in such a manner as to cause 50 to 60% or more of the sulfur present in the pyrite to be discharged as sulfur and the remainder, except that remaining in the cinder or ash, to be discharged as sulfur dioxid. In carrying out this process the gases are passed through the collector Q to remove suspended dust by precipitation as before and are then passed into a retort or furnace D' containing a contact catalyzer such as a mixture of calcium sulfid and calcium sulfite. The temperature of this retort 120

115

120

125

130

is maintained at a red heat by means of gas jets E' fed through the main F'. It is only necessary in carrying out the process in this manner to start the reaction by means of gas jets and heat up the furnace and after once hot and the reaction started maintains the temperature by subsequent reaction, enough natural gas or other hydrocarbon being admitted through the valve in the main F' to 10 decompose the sulfur dioxid. The reaction taking place being as follow:



This reaction occurs indirectly by the 15 breaking down of the calcium sulfite into calcium oxysulfid through the action of the hydrocarbon, and the sulfur dioxid builds the oxysulfid up again to sulfite as follows:



The sulfur is extracted from the sulfur dioxid by removing the oxygen to produce water and carbon dioxid which maintains 25 the temperature. The sulfur set free is vaporized and the sulfur coming from the retort along with the sulfur dioxid simply passes through the furnace. It is therefore evident that this furnace must be air 30 tight or the sulfur would be oxidized.

While in the foregoing I have described a specific apparatus for carrying out the process hereinafter claimed, it is to be understood that the various steps of the process 35 may be carried out by means of other apparatus.

I claim:

1. The herein described process of recovering sulfur from pyritic material which 40 consists in heating the ore whereby to drive off vapors of sulfur dioxid, passing said vapors through a container, heating said container, and finally introducing a gaseous hydrocarbon into the container whereby 45 combustion may take place with the formation of sulfur, carbon dioxid and water.

2. The herein described process of recover-

ing sulfur from pyritic material which consists in heating the ore to drive off sulfur dioxid, passing said sulfur dioxid through a 50 container, heating said container from within through the use of open flame gas jets, and finally introducing illuminating gas into the container whereby combustion may take place in the formation of sulfur, carbon dioxid and water.

3. The herein described process of recovering sulfur from pyritic material which consists in heating the ore to drive off sulfur dioxid, passing said sulfur dioxid through a 60 container, heating said container, and finally passing a gaseous hydrocarbon through said container in the presence of a catalytic agent whereby combustion takes place with the formation of sulfur, carbon dioxid and 65 water.

4. The herein described process of recovering sulfur from pyritic material which consists in heating the ore to drive off sulfur dioxid, passing the sulfur dioxid through a 70 container having therein a mixture of calcium sulfid, and calcium sulfite, heating the interior of the container through the medium of open flame gas jets, and finally passing a gaseous hydrocarbon through said container whereby combustion takes place with 75 the formation of sulfur, carbon dioxid and water.

5. The herein described process for regulating the combustion of pyritic material 80 for the recovery of sulfur therefrom which consists in placing the material in a container which is higher than its width, igniting the material at the bottom thereof, and withdrawing the material from the bottom 85 after combustion has been completed continuously to permit the downward feeding of material toward the heated zone.

In testimony whereof I affix my signature in presence of two witnesses.

ADDISON F. HOFFMAN.

Witnesses:

JENNIE JONES,  
E. D. WRIGLEY.